

(No Model.)

T. B. ATTERBURY.

METHOD OF MANUFACTURING ORNAMENTAL GLASS.

No. 398,995.

Patented Mar. 5, 1889.



WITNESSES.

F. L. Ourand  
H. M. Atterbury.

INVENTOR.

T. B. Atterbury  
By  
E. W. Ginsbach  
Attorney.

# UNITED STATES PATENT OFFICE.

THOMAS B. ATTERBURY, OF PITTSBURG, PENNSYLVANIA.

## METHOD OF MANUFACTURING ORNAMENTAL GLASS.

SPECIFICATION forming part of Letters Patent No. 396,995, dated March 5, 1889.

Application filed September 20, 1888. Serial No. 289,908. (No model.)

To all whom it may concern:

Be it known that I, THOMAS B. ATTERBURY, a citizen of the United States, and a resident of Pittsburg, in the county of Allegheny and State of Pennsylvania, have invented new and useful Improvements in the Method of Manufacturing Ornamental Glass; and I do hereby declare the following to be a full, clear, and exact description of said invention, reference being had to the accompanying drawings, and to the letters or figures of reference marked thereon, which form a part of this specification.

My invention relates to a new and useful method of manufacturing ornamental or decorated glass.

The object of my invention is to provide a simple and inexpensive method of ornamenting glass and glass articles with letters, figures, flowers, vines, stripes, and miscellaneous decorations during the operation of forming the article, thus shaping and decorating the article in colors in one and the same operation.

My invention consists in providing the plate or marver with any suitable design cut therein, said design being filled with one or more metallic oxides or mineral colors or finely-pulverized colored glass, which will adhere to the hot glass bulb and produce a contrast of color from the main body, and in finally finishing the article by blowing in a mold or in any other desirable manner.

Referring to the drawings, Figure 1 is a view in perspective of a plate or marver having the design cut therein and a bulb of glass on the blow-pipe in the act of being rolled over the same. Fig. 2 is also a view in perspective of a plate or marver having grooves cut therein to form articles with stripes of different colors from the main body of the article.

In carrying out my invention I embed and fuse into the partially-formed article metallic oxides or mineral colors, or finely divided or pulverized colored glass, which will produce a contrast of color with the main body when the article is formed.

In producing mottled glassware—i. e., glass-ware having splotches or spots of different colors without any regularity as to form of

design—the metallic oxides or mineral colors or finely-divided colored glass is scattered or sprinkled on a plain metallic plate or marver, and the partially-blown bulb of glass while 55 in a highly-heated or working condition is rolled over it, thus causing the coloring-matter or pulverized glass to adhere to it, after which the bulb is reheated, so as to fuse the oxides or colored glass adhering to it, the 60 bulb being then blown in a mold or otherwise manipulated to form the article.

In forming articles of glassware on which I wish to place ornaments or designs of a pre-determined outline cut into the face of the 65 plate or marver A the ornament of the configuration desired, which may be in representation of fruits, flowers, vines, leaves, beasts, birds, reptiles, &c., and fill said depressed portions of the marver with metallic 70 oxides, mineral colors, or finely-pulverized colored glass or vitrifiable material. Instead of making the design in depression on the marver, I may use a plain smooth plate on which the design is printed in metallic colors 75 by means of a rubber block on which the design has been made; or stencil-plates having the desired design cut therein may be used to apply the metallic colors to the marver, said colors being mixed with oil or turpentine, 80 so as to be more readily applied, the oil or turpentine being consumed as soon as it comes in contact with the hot glass bulb.

The operator now gathers on his blow-pipe or punti a bulb of glass, B, which he partially 85 expands by blowing, and then rolls the same over the marver, while hot, from one side to the other. The coloring-matter in the recesses or cavities or on the surface of the marver adheres to the glass on the blow-pipe, and thus 90 transfers the exact design or ornamentation to the bulb. This bulb of glass is now reheated and blown in a mold or otherwise worked to form the article, when it will be found that the ornamental design on the plate 95 or marver will be produced in contrasting colors on the article.

If the article is to be pressed, the reheating of the bulb is not required, for the reason that the thick unblown bulb as it comes from the pot has sufficient heat to fuse the colors 100 without reheating, and after the bulb has

been rolled on the marver to take up the colors it is put in the press-mold and severed from the blow-pipe and pressed in the usual manner.

5 For fine decorations or ornamentations I prefer to use metallic oxides or mineral colors, for the reason that in the reheating they melt smooth and give a more artistic effect; but good effects can be produced by the use of 10 finely-pulverized colored glass, and the colored glass may be used separately or mixed, and metallic oxides or mineral colors may also be mixed with the powdered glass, so as to produce beautiful effects in tints and 15 shades of color.

It will be seen that by the above-described method of ornamentation I can readily and cheaply form names, letters, figures, monograms, bands, stripes, and all manner of decorations on the articles while the same are being formed into the shape desired, thus dispensing with hand-painting and the subsequent firing to fuse the colors on the article, as is now the common practice. It will also be 25 noticed that window-glass for churches and for other architectural purposes can be made in the same manner, the cylinders from which the sheet-glass is formed being rolled, while hot, over the marver on which the coloring-matter is deposited, after which the cylinder 30 is reheated, split, and flattened in the manner usually practiced in making window-glass.

The method herein described may be varied without departing from the spirit of my invention—for example, the design on the plate or marver may be raised or in relief, and the coloring-matter placed on the plain or depressed portions of the marver. This would 35 produce the design in plain colors, or of the

color of the main body of the glass, while the 40 other portions of the article would appear in mottled work or in contrasting colors, as the case may be.

I am aware that it is not new to impress upon the surface of the powdered substances 45 upon which the sheet-glass is to be placed a suitable design, so that when the glass placed upon it becomes softened by the action of the heat the glass may embed itself into the cavities of the design and so produce an embossed 50 or raised surface dead or bright, as may be desired, and such I do not claim.

Having thus described my invention, what I claim is—

1. The herein-described improvement in the 55 art of manufacturing ornamental glass, which consists in rolling the glass bulb or ball, while in a hot condition, on a plate or marver having the design formed thereon, on which is placed a vitrifiable coloring material, and 60 finally shaping the bulb into the article desired.

2. The herein-described improvement in the art of manufacturing ornamental glass-ware, which consists in rolling the hot bulb or ball 65 of glass over a marver having a design formed thereon of vitrifiable coloring material such as described, thus depositing the colors on the bulb, reheating the bulb to fuse the colors, and finally blowing or pressing the bulb in a mold 70 to form the article, as set forth.

In testimony whereof I affix my signature in presence of two subscribing witnesses.

THOMAS B. ATTERBURY.

Witnesses:

D. P. BERG,  
G. STENGEL.